

## UNITED STATES PATENT OFFICE

2,135,092

## BUILT-UP LUBRICATING OIL

George M. Maverick, Elizabeth, N. J., assignor  
to Standard Oil Development Company, a cor-  
poration of Delaware

No Drawing. Application December 20, 1933,  
Serial No. 703,213

9 Claims. (Cl. 87—9)

The present invention relates to an improved lubricating oil, and especially to an oil for the lubrication of internal combustion engines or for similar service. The invention will be fully understood from the following description of the lubricant and its method of production.

Lubricating oils for use in internal combustion engines are subjected to extremely severe service and it has been fortunate that the naturally occurring oils have accidentally been endowed with properties suitable for such service, if only in an imperfect degree. Recent studies of the several attributes desired for lubricating internal combustion engines have made it evident that several separate properties are desired for accomplishing different purposes and are so diverse as not to be possessed to any marked degree by any single class of substances. If a lubricant is chosen for its superior qualities in one respect, it has been found to be proportionately lacking in some other respect which is equally desirable. Even at present the best lubricating oils hold their place by a compromise; in other words, hydrocarbon lubricating oils have none of the desired attributes to a very high degree and are suitable only because they show all of the desired attributes albeit, to a rather low degree.

In the present invention the problem of lubricating automotive engines is attacked from an entirely different point of view, by selecting and mixing several different ingredients, each selected to serve a particular purpose, so that it has been possible to produce oils in this manner which are markedly superior to natural or modified natural lubricants. It has been found that by compounding the individual ingredients for the several different purposes, the various properties desired can be obtained to an extremely high degree and that while no single ingredient possesses all of the characteristics desired, the different constituents are so chosen and mixed in such proportions as to supply the desired properties with any particular emphasis desired and to greatly minimize undesirable properties.

The present oils are prepared by first selecting a suitable vehicle or base, the primary purpose of which is to carry the several substances added in a fluid form capable of easy flow through the engine. This vehicle is preferably a highly purified hydrocarbon oil of low to medium viscosity, that is to say, generally lower than the viscosity now used for lubricating automotive engines. For example, it may be free from 40-50 seconds Saybolt at 210° F. The oil is sufficiently high boiling to give it a suitable flash point of, say,

400°-450° and it is preferably closely cut. It should be well refined by any of the known methods and be free from carbon forming substances—asphaltenes, resins and the like. Such an oil is preferably purified to such a degree by acid treatment, hydrogenation, solvent extraction or the like that it is characterized by a higher rate of oxidation than the crude cut from which it is derived. The so-called "white" mineral oils can be used for this purpose as well as synthetic lubricating oils prepared by condensation of cracked oils or waxes, or other active derivatives such as halides. It has also been found that the lighter fractions of lubricating oils prepared by destructive hydrogenation at relatively low temperatures, say from 700°-800° F., whereby they are substantially completely saturated, are also excellent for the present purpose. The vehicle may be a waxy oil or a dewaxed oil or derived from wax free crudes. If a waxy oil is used, a pour inhibitor may be added.

To the vehicle described above is then added a thickening agent and for this purpose natural, modified natural, or synthetic linear hydrocarbon polymers are the most desirable; for example, polymerization products of alpha olefines, particularly of isobutylene are highly desirable. These materials are polymerized by the action of active clay, carbon, or the well-known halide catalysts especially aluminum chloride and boron fluoride. Other materials may also be used, such as polymerized indene, styrene or the like or their alkylated or hydrogenated polymerized products, as well as condensation products of dihalo hydrocarbons of less than five carbon atoms with single ringed aromatic hydrocarbons, namely, ethylene dichloride with benzol. Natural materials such as rubber are also suitable but hydrogenated products are much more desirable. The hydrogenated products of related materials such as the balatas, guttas, and guayule may also be used. The amount of thickener to be used depends on its molecular weight and the viscosity of the product desired. If a high molecular weight polymer is selected, less is required to produce a given thickening effect than if a lower polymer is employed. In general, however, the amount varies between, say, 1-10% by weight of the vehicle. These thickeners increase the viscosity well above 50 seconds Saybolt at 210° F.; for example, 60, 75, or over 100 seconds at 210° F. as desired. In this way, irrespective of the particular vehicle, it is possible to produce all of the grades of motor lubricants by varying the amount of the polymer added.

These thickening agents not only have the property of increasing viscosity but also the desirable property of decreasing the slope of the viscosity-temperature curve, or in other words of increasing the viscosity index of the blend.

The second essential substance to be added to the base stock is an oxidation inhibitor. These substances are well known and any reasonably good inhibitor will serve the present purpose; for example, phenolic or preferably cresolic substances—the mono-, di-, and hydroxy benzols or cresols. The naphthols—alpha and beta—or the naphthylamines may also be used. Sulfur compounds are useful, for example, aromatic disulfides, mercaptans or polysulfides, whether aromatic or aliphatic, and especially the trisulfides which are non-corrosive. These substances are merely mentioned as examples to indicate the class or nature of the materials to be used for the present purpose. The amount used varies with the potency of the particular inhibitor but in general they may be used in amounts from .01-.05 to .1% or even up to 1% or more.

The third essential ingredient is a substance from the class of the sludge dispersers. The action of these materials is obscure but they appear to maintain oxidation products of the oil in a state of suspension, checking to a marked extent the polymerization or agglomeration and precipitation on the hot portions of the engine, especially the valves, rings, pistons and in the crankcase. The substances themselves, whatever their action may be, comprise the class of synthetic hydrocarbons of high boiling point, so high in fact that they are to be classed as substantially undistillable. They are in addition rich in hydrogen, the carbon-hydrogen ratio closely approaching that characteristic of the paraffin series of hydrocarbons. They must also be free flowing liquids. Substances of the type mentioned above may be prepared synthetically by condensing hydrocarbon waxes or paraffin oils, which are themselves as close as possible to being completely saturated. The high molecular weight initial materials are more desirable than the lower, for example, a condensation product of petrolatum is ordinarily to be preferred to a condensation product of a low molecular weight wax. Condensation may be accomplished in any convenient manner, for example, by subjecting the oil or wax to high voltage, high frequency alternating electric discharges or by more strictly chemical means, for example, by chlorinating and subsequently condensing the chlorinated hydrocarbons during which reaction hydrochloric acid is removed. Condensation should not proceed so far as to produce rubbery insoluble substances but readily soluble or dispersible materials. This can readily be accomplished by adjusting the time of reaction. Olefines derived from waxy hydrocarbons may also be condensed, preferably using aluminum chloride or very similar condensation catalysts. Cracked waxes or cracked paraffin oils furnish a good source of condensable materials which yield substantially saturated polymers. If desired, a relatively small amount of an aromatic hydrocarbon may be added during condensation, for example, 5-10%, in order to furnish condensation nuclei, although it should be understood that this is not required and even where used the products still closely approach the carbon-hydrogen ratio of saturated hydrocarbons.

The amount of the sludge dispersing substances varies with their particular potency. Ordinarily

1% is sufficient, but this amount may be increased to 2% or 3% where less active substances are used. There is a definite optimum quantity which if exceeded shows less dispersing power. The preferred amount is so small as to show no very substantial increase in the viscosity of the blend as measured at 210° F. For example, the increase in viscosity due to the sludge dispersing agent is generally not more than 2-4 seconds Saybolt at 210° F.

10 While the hydrocarbon materials listed above are preferred, it is possible to use oxygen-containing substances, for example, polymers of high boiling acids, ethers, ketones, esters and the like or fatty substances, prepared by the action of 15 high frequency, high voltage, electric discharges or other known means. Ordinarily these are used in larger amounts than the best hydrocarbon dispersing agents.

10 In order to produce a lubricant with a high 20 degree of oiliness, friction reducing agents may be added. These may be selected from the various types now known—fatty oils, fatty acids, or higher alcohols may be used—but it is preferred to use highly purified esters, particularly those 25 synthetically prepared, so as to avoid the presence of non-fats, unstable gummy materials and the like which are always contained to a more or less substantial degree in natural esters either animal or vegetable. Esters boiling above 150° or 30 200° C. are preferred, since they will not be lost from the hot oil and may be prepared from naturally occurring acids such as stearic or oleic or from acids obtained by the oxidation of paraffin wax, particularly at low temperatures, with air. 35 The methyl, ethyl, and propyl esters of these acids are very satisfactory and are to be preferred to the higher alkyl esters. The amount of the ester is ordinarily from .5 to 5%. The presence of these friction reducing agents greatly 40 increases the load bearing capacity of the oil and reduces the friction in the bearings.

45 Other agents besides the esters mentioned above may be used to increase bearing pressures and to reduce friction; for example, sulfurized bases, chlorin-containing organic materials in relatively small amounts, or substances containing both chlorin and sulfur in the same molecule, or if desired in separate substances. Soaps of the alkali or alkaline earth or heavy metals such as 50 lead and zinc, may be used in small amounts.

55 Material of the type of carbon preventers may be added, if desired. These materials are distinguished from the sludge dispersers, in that they show little or no effect on Sligh numbers, and are, perhaps, misnamed in that they probably do not actually decrease the amount of carbon formed. Their action is rather to influence the type of carbon rendering it soft and fluffy rather than flinty and adherent.

60 The amount of carbon retained within the engine is influenced by these so-called preventers. High boiling soluble esters such as butyl, amyl, hexyl phthalates, benzoates, salicylates or amines of the same general boiling range are used. These 65 may be used in amounts up to 1% or 2% but generally not over about 5 to 10%.

70 In addition to the ingredients mentioned above, other various materials may be added such as pour inhibitors if a waxy vehicle is originally employed or if waxy materials are added for any reason. The preferred pour inhibitors are hydrocarbons produced by low temperature aluminum chloride or high frequency electrical con- 75

5 densation of hydrocarbon waxes, either alone or in presence of aromatics.

The following formulae are given to illustrate the composition of the improved lubricating oils.

5

**I**

As a vehicle a highly refined mineral oil of the following inspection is selected:

10 Gravity degrees A. P. I. 28.7  
 Viscosity at 100° F. seconds Saybolt 265  
 Viscosity at 210° F. do 50  
 Flash 410  
 Pour point degrees Fahrenheit 25  
 Sigh test (2½ hr.) 10.5

15 To 100 parts by weight of the vehicle is added two parts of a substance prepared by the polymerization of isobutylene at -20° F. with boron fluoride. To parts of an isopropyl ester of acids produced by the air oxidation of paraffin wax is 20 also added together with one part of a condensation product of petrolatum (chlorinated to about 12%) with 10% of naphthalene and as an oxidation inhibitor .05% of alpha naphthol. The finished composition is an excellent medium grade 25 motor lubricant extremely resistant to oxidation with a very low tendency to sludge and high oiliness. It is excellently adapted to the breaking in of new or "green" motors.

30

**II**

In a second composition a similar vehicle is used which has been prepared by destructive hydrogenation of heavier oils at a temperature of 700-800° F. and under pressures of 200 atmospheres whereby the oil is substantially completely saturated. To 100 parts of the oil vehicle is added 3 parts of hydrogenated rubber together with 2½ parts of ethyl oleate, which serves as an anti-friction agent. One part of a condensation product of petrolatum produced by the action of high frequency alternating electric discharges is added 40 as a dispersing agent and as the oxidation inhibitor .1% of naphthyl disulfide is employed.

45

**III**

To an oil vehicle similar to that used in Example II are added the same thickening polymer together with a .05% of alpha thio naphthol as an oxidation inhibitor and a sludge disperser of the 50 type and in the amount used in Example I.

**IV**

To 100 parts of vehicle similar to that used in Example I but with a viscosity of 60 seconds at 55 210° F. is added 2 parts of a polymer produced by the polymerization of isobutylene with boron fluoride. This polymer is of considerably lower molecular weight than that used in Example I and produces an oil with a viscosity of 70 seconds 60 Saybolt at 210° F. To the composition is added .5 part of an inhibitor prepared by treating a high boiling mercaptan with sodium plumbite and sulfur, 1 part of the disperser used in Example I and +5% dibutyl phthalate as carbon preventer.

65

**V**

To the oil last described is added a small quantity, about 2%, of a substance prepared by chlorinating paraffin wax and reacting the same with 70 sodium polysulfide so as to obtain a final product containing sulfur but free from chlorine which gives the oil extreme pressure bearing properties.

In the above compositions the nature and the

amount of the various ingredients may vary to suit particular conditions to be met and it is possible to make a full and complete line of motor oils or oils for other, similar purposes by adjusting the composition of the blends as 5 brought out in the previous examples.

My invention is not to be limited to the use of particular compositions shown, nor to any particular ingredient, but only to the following claims in which it is desired to claim all novelty 10 inherent in the invention.

I claim:

1. An improved lubricant, comprising a vehicle which is a high boiling hydrocarbon oil of viscosity lower than that ordinarily used for lubricating purposes, a thickening polymer of the linear hydrocarbon type, an oxidation inhibitor and a sludge disperser. 15

2. An improved lubricant, comprising a hydrocarbon oil vehicle of viscosity below the lubricating range, a thickening polymer selected from the group comprising polymerized isobutylene, hydrogenated rubber, and the condensation products of di-halo hydrocarbons of less than five carbon atoms condensed with mono-cyclic 25 aromatic hydrocarbons, an oxidation inhibitor and a sludge disperser.

3. An improved motor lubricant, comprising a high boiling hydrocarbon vehicle of less viscosity than used for lubricating purposes, a thickening 30 polymer and a dispersing agent comprising a high boiling synthetic hydrocarbon condensation product, free flowing and having a carbon-hydrogen ratio closely approaching that of the paraffin series, and an oxidation inhibitor. 35

4. An oil according to claim 3 in which the thickening polymer is produced from isobutylene.

5. An oil according to claim 3 in which the sludge disperser is obtained by condensation of waxy hydrocarbons and is used in the proportion 40 of about 1%.

6. An oil according to claim 3 in which the sludge disperser is obtained by the condensation of waxy hydrocarbons on an aromatic nucleus and is used in the proportion of about 1%. 45

7. Oil according to claim 3 in which a small amount of an organic ester boiling about 150° C. is added.

8. A lubricant of suitable viscosity for the lubrication of motors, having a high resistance to oxidation and concomitantly a low tendency to deposit sludge, comprising a hydrocarbon oil vehicle of lower viscosity, a sufficient amount of a thickening agent of the polymer type to bring the viscosity of the vehicle to that desired in the motor oil, an effective amount of an oxidation inhibitor and an effective amount of an agent capable of maintaining sludge in suspension. 55

9. A lubricant of suitable viscosity for the lubrication of motors, having a high resistance to oxidation and concomitantly a low tendency to deposit sludge, comprising a high boiling hydrocarbon oil obtained by purification of crude oil and having a viscosity lower than that desired in the finished lubricant, a sufficient amount of a thickening polymer of the linear hydrocarbon type to bring the viscosity of the hydrocarbon oil to that desired in the finished lubricant, an effective amount of an oxidation inhibitor and an effective amount of an agent capable of maintaining sludge in suspension in said oil. 60